

## UNITED STATES PATENT OFFICE

LEON R. WESTBROOK, OF CLEVELAND HEIGHTS, OHIO, ASSIGNOR, BY MESNE ASSIGNMENTS, TO THE GRASSELLI CHEMICAL COMPANY, OF CLEVELAND, OHIO, A CORPORATION OF DELAWARE

## ELECTROPLATING

No Drawing.

Application filed February 23, 1928. Serial No. 256,493.

This invention relates to addition agents to be used in cadmium-cyanide electroplating baths, and the novel plating baths obtained thereby.

The production of bright, adherent, commercially useful cadmium plates on steel or other metals presents a number of difficulties which have usually been solved by the use, in connection with the cyanide plating baths, of a brightening agent and an organic addition agent.

Practically all addition agents which so far have been found to be beneficial in their action are of a more or less colloidal organic nature and of ill defined and possibly varying composition so that it is sometimes difficult to determine from a chemical analysis if a given material will produce constant and reproducible results in an electroplating bath.

I have now found that certain so-called dyestuff intermediates which are commercially available in constant and analytically determinable purity are particularly suited as addition agents to electroplating baths. They are naphthalene compounds which couple with diazo compounds and are of an acidic nature, and my preferred addition agents are chemically distinguished by being compounds in which the naphthalene nucleus is substituted by an acidic radical such as the sulfo or carboxylic group and by an amino or hydroxy group or both the latter. It is, of course, necessary that such compounds be water soluble, or soluble in the cadmium-cyanide bath.

My novel cadmium plating baths are produced by dissolving in water a cadmium compound, a cyanide, other electrolytes required to promote the electrodeposition of cadmium, and a small amount of a naphthalene compound containing an acidic group and being capable of coupling with a diazo compound. Amongst the other electrolytes re-

quired to promote the deposition of commercially valuable chromium plates, I refer particularly to the so-called brightening agents by which I mean the nickel or copper salts as disclosed in my Patent No. 1,681,509, 50 granted August 21, 1928.

Such a plating bath is then used in the conventional manner at the usual temperatures and current densities. The plates obtained are, however, superior in brightness 55 and adhesiveness to those obtained from a similar bath in which the addition agent has been omitted.

A typical representative of such a novel bath is obtained by dissolving in water, to 60 1 liter, the following:

|                                      | Grams |
|--------------------------------------|-------|
| NaCN                                 | 120   |
| Cd(OH) <sub>2</sub>                  | 48    |
| Na <sub>2</sub> SO <sub>4</sub>      | 60    |
| NiSO <sub>4</sub> ·7H <sub>2</sub> O | 65    |
|                                      | 1     |

10 to 15 grams of one of my novel addition agents or a mixture of such agents is then dissolved in this bath and, using a cadmium anode and the article to be plated as the cathode, the current is passed through the bath at the usual temperatures and current densities.

Typical representatives of the class of 75 naphthalene compounds which I found to be most useful as addition agents are represented by the following:

H acid (1-8-amino-naphthol-3-6-disulfonic acid).

F acid (betanaphthylamine monosulfonic acid).

Cleves acids (1-6 and 1-7 naphthylamine-sulfonic acid).

Laurents acid (1-5-naphthylamine-sulfonic acid).

Gamma acid (2-amino-8-naphthol-6-sulfonic acid).

Neville-Winther acid (1-4-naphthol-sulfonic acid).

Naphthionic acid (1-4-naphthylamine-sulfonic acid).

G salt (sodium-beta-naphthol-6-8-disulfonate).

It is well known that these compounds will easily couple in aqueous solution with aromatic diazo compounds.

Amongst these I found the naphthylamine monosulfonic acids, such as the F, Cleves, 10 and Laurents acids, to have the most beneficial effect.

It is immaterial whether the free acids or their water soluble salts are dissolved in the cadmium cyanide bath, and both can, for 15 purposes of this invention, be considered entirely equivalent.

I claim:

1. An electroplating bath comprising an aqueous solution containing a cadmium 20 pound, a cyanide, a brightening agent, and an acidic naphthalene compound capable of coupling with a diazo compound.

2. An electroplating bath comprising an aqueous solution containing a cadmium 25 pound, a cyanide, a brightening agent, and a naphthalene sulfonic acid compound capable of coupling with a diazo compound.

3. An electroplating bath comprising an aqueous solution containing a cadmium 30 pound, sodium cyanide, a brightening agent, and a naphthylamine monosulfonic acid compound.

4. An addition agent for cadmium cyanide electroplating baths comprising an acidic 35 naphthalene compound capable of coupling with a diazo compound.

5. An addition agent for cadmium cyanide electroplating baths comprising a naphthalene sulfonic acid compound capable 40 of coupling with a diazo compound.

6. An addition agent for cadmium cyanide electroplating baths comprising a naphthylamine sulfonic acid compound.

7. An electroplating bath comprising an 45 aqueous solution containing a cadmium compound, a cyanide, and an acidic naphthalene compound capable of coupling with a diazo compound.

8. The process of producing bright adherent cadmium plates which comprises electrodepositing cadmium from an aqueous 50 solution containing a cadmium compound, a cyanide, and an acidic naphthalene compound capable of coupling with a diazo compound.

9. The process of producing bright adherent cadmium plates which comprises electrodepositing cadmium from an aqueous 55 solution containing a cadmium compound, a cyanide, a brightening agent, and an acidic naphthalene compound capable of coupling with a diazo compound.

10. The process of producing bright adherent cadmium plates which comprises 60 electrodepositing cadmium from an aqueous

solution containing a cadmium compound, a cyanide, a brightening agent, and a naphthalene sulfonic acid compound capable of coupling with a diazo compound.

11. The process of producing bright adherent cadmium plates which comprises electrodepositing cadmium from an aqueous 70 solution containing a cadmium compound, sodium cyanide, a brightening agent, and a naphthylamine monosulfonic acid compound. 75

In testimony whereof, I affix my signature.

LEON R. WESTBROOK.

80

85

90

95

100

105

110

115

120

125

130